



US008029956B2

(12) **United States Patent**  
**Qi et al.**

(10) **Patent No.:** **US 8,029,956 B2**  
(45) **Date of Patent:** **Oct. 4, 2011**

(54) **PHOTORECEPTOR WITH OVERCOAT LAYER**

(75) Inventors: **Yu Qi**, Oakville (CA); **Hany Aziz**, Oakville (CA); **Nan-Xing Hu**, Oakville (CA); **Ah-Mee Hor**, Mississauga (CA); **Kenny-Tuan Dinh**, Webster, NY (US); **John F Yanus**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 459 days.

(21) Appl. No.: **11/275,546**

(22) Filed: **Jan. 13, 2006**

(65) **Prior Publication Data**

US 2007/0166634 A1 Jul. 19, 2007

(51) **Int. Cl.**  
**G03G 5/047** (2006.01)

(52) **U.S. Cl.** ..... **430/58.7**; 430/58.05; 430/66; 430/132  
(58) **Field of Classification Search** ..... 430/58.75,  
430/58.05, 58.7, 66, 132

See application file for complete search history.

(56) **References Cited**

U.S. PATENT DOCUMENTS

|               |         |                              |
|---------------|---------|------------------------------|
| 3,121,006 A   | 2/1964  | Middleton et al.             |
| 4,050,935 A   | 9/1977  | Limburg et al.               |
| 4,181,526 A * | 1/1980  | Blakey et al. .... 430/67    |
| 4,281,054 A   | 7/1981  | Horgan et al.                |
| 4,297,425 A   | 10/1981 | Pai et al.                   |
| 4,298,697 A   | 11/1981 | Baczec et al.                |
| 4,338,390 A   | 7/1982  | Lu                           |
| 4,355,154 A * | 10/1982 | Saam et al. .... 528/274     |
| 4,457,994 A   | 7/1984  | Pai et al.                   |
| 4,560,635 A   | 12/1985 | Hoffend et al.               |
| 4,599,286 A   | 7/1986  | Limburg et al.               |
| 4,871,634 A   | 10/1989 | Limburg et al.               |
| 5,368,967 A   | 11/1994 | Schank et al.                |
| 5,418,107 A   | 5/1995  | Nealey et al.                |
| 5,456,989 A * | 10/1995 | Nogami et al. .... 430/58.05 |

|                   |         |                                 |
|-------------------|---------|---------------------------------|
| 5,681,679 A       | 10/1997 | Schank et al.                   |
| 5,702,854 A       | 12/1997 | Schank et al.                   |
| 5,709,974 A       | 1/1998  | Yuh et al.                      |
| 5,976,744 A       | 11/1999 | Fuller et al.                   |
| 6,004,709 A       | 12/1999 | Renfer et al.                   |
| 6,010,810 A *     | 1/2000  | Uesaka et al. .... 430/58.8     |
| 6,103,436 A       | 8/2000  | Yanus et al.                    |
| 7,384,717 B2 *    | 6/2008  | Dinh et al. .... 430/66         |
| 7,759,032 B2 *    | 7/2010  | Yanus et al. .... 430/66        |
| 2001/0044060 A1 * | 11/2001 | Shida et al. .... 430/58.2      |
| 2002/0052451 A1 * | 5/2002  | Vandevoorde et al. .... 525/533 |
| 2003/0082468 A1 * | 5/2003  | Hu et al. .... 430/58.7         |
| 2005/0064337 A1 * | 3/2005  | Suganuma et al. .... 430/300    |
| 2005/0266325 A1 * | 12/2005 | Yanagawa et al. .... 430/58.7   |
| 2007/0072101 A1 * | 3/2007  | Dinh et al. .... 430/66         |
| 2007/0134573 A1 * | 6/2007  | Yanus et al. .... 430/66        |

FOREIGN PATENT DOCUMENTS

|    |              |        |
|----|--------------|--------|
| EP | 0 660 191 A1 | 6/1995 |
| EP | 1 014 205 A2 | 6/2000 |
| EP | 1 174 771 A1 | 1/2002 |

OTHER PUBLICATIONS

U.S. Appl. No. 11/234,275, filed Jun. 25, 2005, Dinh et al.  
U.S. Appl. No. 11/295,134, filed Dec. 13, 2005, Yanus et al.

\* cited by examiner

Primary Examiner — Mark F Huff

Assistant Examiner — Rachel Zhang

(74) Attorney, Agent, or Firm — Oliff & Berridge, PLC

(57) **ABSTRACT**

An electrophotographic imaging member includes a substrate, a charge generating layer, a charge transport layer, and an overcoating layer, the overcoating layer being a cured film formed from a film forming resin composition including at least a melamine compound, a polyol, and a charge transport compound, where the charge transport compound is represented by:



where Q represents a charge transport component, L represents a divalent linkage group, and n represents a number of repeating segments or groups.

**12 Claims, No Drawings**

## PHOTORECEPTOR WITH OVERCOAT LAYER

## TECHNICAL FIELD

This disclosure is generally directed to electrophotographic imaging members and, more specifically, to layered photoreceptor structures with an improved overcoat layer. In particular, this disclosure relates to electrophotographic imaging members with an improved overcoat layer comprising, as a hole transporting molecule, a hydroxyl-containing hole transport compound. This disclosure also relates to processes for making and using the imaging members.

## RELATED APPLICATIONS

Copending U.S. patent application Ser. No. 11/234,275 filed Sep. 26, 2005, discloses an electrophotographic imaging member comprising: a substrate, a charge generating layer, a charge transport layer, and an overcoating layer, said overcoating layer comprising a cured polyester polyol or cured acrylated polyol film forming resin and a charge transport material.

U.S. patent application Ser. No. 11/275,134 filed Dec. 13, 2005 (now U.S. Pat. No. 7,759,032), discloses an electrophotographic imaging member comprising: a substrate, a charge generating layer, a charge transport layer, and an overcoating layer, said overcoating layer comprising a terphenyl arylamine dissolved or molecularly dispersed in a polymer binder.

The appropriate components and process aspects of the foregoing, such as the imaging member composition, components and methods, may be selected for the present disclosure in embodiments thereof. The entire disclosures of the above-mentioned application is totally incorporated herein by reference.

## REFERENCES

Various overcoats employing alcohol soluble polyamides have been proposed in the prior art. One of the earliest ones is an overcoat comprising an alcohol soluble polyamide without any methyl methoxy groups (Elvamide) containing N,N'-diphenyl-N,N'-bis(3-hydroxyphenyl)-[1,1'-biphenyl]-4,4'-diamine. This overcoat is described in U.S. Pat. No. 5,368,967, the entire disclosure thereof being incorporated herein by reference. Although this overcoat had very low wear rates in machines employing corotrons for charging, the wear rates were higher in machines employing BCR. A cross linked polyamide overcoat overcame this shortcoming. This overcoat comprised a cross linked polyamide (e.g. Luckamide) containing N,N'-diphenyl-N,N'-bis(3-hydroxyphenyl)-[1,1'-biphenyl]-4,4'-diamine. In order to achieve cross linking of the polyamide polymer, Luckamide, having methyl methoxy groups was employed along with a catalyst such as oxalic acid. This tough overcoat is described in U.S. Pat. No. 5,702,854, the entire disclosure thereof being incorporated herein by reference. With this overcoat, very low wear rates were obtained in machines employing bias charging rolls (BCR) and Bias Transfer Rolls (BTR). Durable photoreceptor overcoatings containing cross linked polyamide (e.g. Luckamide) containing N,N'-diphenyl-N,N'-bis(3-hydroxyphenyl)-[1,1'-biphenyl]-4,4'-diamine (DHTBD) (Luckamide-DHTBD) have been prepared using oxalic acid and trioxane to improve photoreceptor life by at least a factor of 3 to 4. Such improvement in the bias charging roll (BCR) wear resistance involved crosslinking of Luckamide under heat treatment, e.g. 110°

C.-120° C. for 30 minutes. However, adhesion of this overcoat to certain photoreceptor charge transport layers, containing certain polycarbonates (e.g., Z-type 300) and charge transport materials (e.g., bis-N,N-(3,4-dimethylphenyl)-N-(4-biphenyl)amine and N,N'-diphenyl-N,N'-bis(3-methylphenyl)-[1,1'-biphenyl]-4,4'-diamine) is greatly reduced under such drying conditions. On the other hand, under drying conditions of below about 110° C., the overcoat adhesion to the charge transport layer was good, but the overcoat had a high rate of wear. Thus, there was an unacceptably small drying conditions window for the overcoat to achieve the targets of both adhesion and wear rate.

U.S. Pat. No. 5,702,854 describes an electrophotographic imaging member including a supporting substrate coated with at least a charge generating layer, a charge transport layer and an overcoating layer, said overcoating layer comprising a dihydroxy arylamine dissolved or molecularly dispersed in a crosslinked polyamide matrix. The overcoating layer is formed by crosslinking a crosslinkable coating composition including a polyamide containing methoxy methyl groups attached to amide nitrogen atoms, a crosslinking catalyst and a dihydroxy amine, and heating the coating to crosslink the polyamide. The electrophotographic imaging member may be imaged in a process involving uniformly charging the imaging member, exposing the imaging member with activating radiation in image configuration to form an electrostatic latent image, developing the latent image with toner particles to form a toner image, and transferring the toner image to a receiving member.

U.S. Pat. No. 5,681,679 discloses a flexible electrophotographic imaging member including a supporting substrate and a resilient combination of at least one photoconductive layer and an overcoating layer, the at least one photoconductive layer comprising a hole transporting arylamine siloxane polymer and the overcoating comprising a crosslinked polyamide doped with a dihydroxy amine. This imaging member may be utilized in an imaging process including forming an electrostatic latent image on the imaging member, depositing toner particles on the imaging member in conformance with the latent image to form a toner image, and transferring the toner image to a receiving member.

U.S. Pat. No. 6,004,709 discloses an allyloxy polyamide composition, the allyloxy polyamide being represented by a specific formula. The allyloxy polyamide may be synthesized by reacting an alcohol soluble polyamide with formaldehyde and an allyl alcohol. The allyloxy polyamide may be cross linked by a process selected from the group consisting of (a) heating an allyloxy polyamide in the presence of a free radical catalyst, and (b) hydrosilation of the double bond of the allyloxy group of the allyloxy polyamide with a silicon hydride reactant having at least 2 reactive sites. A preferred article comprises a substrate, at least one photoconductive layer, and an overcoat layer comprising a hole transporting hydroxy arylamine compound having at least two hydroxy functional groups, and a cross linked allyloxy polyamide film forming binder. A stabilizer may be added to the overcoat.

U.S. Pat. No. 5,976,744 discloses an electrophotographic imaging member including a supporting substrate coated with at least one photoconductive layer, and an overcoating layer, the overcoating layer including a hydroxy functionalized aromatic diamine and a hydroxy functionalized triarylamine dissolved or molecularly dispersed in a crosslinked acrylated polyamide matrix, the hydroxy functionalized triarylamine being a compound different from the polyhydroxy functionalized aromatic diamine. The overcoating layer is formed by coating. The electrophotographic imaging member may be imaged in a process.

U.S. Pat. No. 5,709,974 discloses an electrophotographic imaging member including a charge generating layer, a charge transport layer and an overcoating layer, the transport layer including a charge transporting aromatic diamine molecule in a polystyrene matrix and the overcoating layer including a hole transporting hydroxy arylamine compound having at least two hydroxy functional groups and a polyamide film forming binder capable of forming hydrogen bonds with the hydroxy functional groups of the hydroxy arylamine compound. This imaging member is utilized in an imaging process.

U.S. Pat. No. 5,368,967 discloses an electrophotographic imaging member comprising a substrate, a charge generating layer, a charge transport layer, and an overcoat layer comprising a small molecule hole transporting arylamine having at least two hydroxy functional groups, a hydroxy or multihydroxy triphenyl methane and a polyamide film forming binder capable of forming hydrogen bonds with the hydroxy functional groups the hydroxy arylamine and hydroxy or multihydroxy triphenyl methane. This overcoat layer may be fabricated using an alcohol solvent. This electrophotographic imaging member may be utilized in an electrophotographic imaging process. Specific materials including Elvamide polyamide and N,N'-diphenyl-N,N'-bis(3-hydroxyphenyl)-[1,1'-biphenyl]-4,4'-diamine and bis-[2-methyl-4-(N-2-hydroxyethyl-N-ethyl-aminophenyl)-]phenylmethane are disclosed in this patent.

U.S. Pat. No. 4,871,634 discloses an electrostatographic imaging member which contains at least one electrophotocductive layer, the imaging member comprising a photo-generating material and a hydroxy arylamine compound represented by a certain formula. The hydroxy arylamine compound can be used in an overcoating with the hydroxy arylamine compound bonded to a resin capable of hydrogen bonding such as a polyamide possessing alcohol solubility.

U.S. Pat. No. 4,297,425 discloses a layered photosensitive member comprising a generator layer and a transport layer containing a combination of diamine and triphenyl methane molecules dispersed in a polymeric binder.

U.S. Pat. No. 4,050,935 discloses a layered photosensitive member comprising a generator layer of trigonal selenium and a transport layer of bis(4-diethylamino-2-methylphenyl) phenylmethane molecularly dispersed in a polymeric binder.

U.S. Pat. No. 4,457,994 discloses a layered photosensitive member comprising a generator layer and a transport layer containing a diamine type molecule dispersed in a polymeric binder and an overcoat containing triphenyl methane molecules dispersed in a polymeric binder.

U.S. Pat. No. 4,281,054 discloses an imaging member comprising a substrate, an injecting contact, or hole injecting electrode overlying the substrate, a charge transport layer comprising an electrically inactive resin containing a dispersed electrically active material, a layer of charge generator material and a layer of insulating organic resin overlying the charge generating material. The charge transport layer can contain triphenylmethane.

U.S. Pat. No. 4,599,286 discloses an electrophotographic imaging member comprising a charge generation layer and a charge transport layer, the transport layer comprising an aromatic amine charge transport molecule in a continuous polymeric binder phase and a chemical stabilizer selected from the group consisting of certain nitrone, isobenzofuran, hydroxyaromatic compounds and mixtures thereof. An electrophotographic imaging process using this member is also described.

U.S. Pat. No. 5,418,107 discloses a process for fabricating an electrophotographic imaging member including providing

a substrate to be coated, forming a coating comprising photoconductive pigment particles having an average particle size of less than about 0.6 micrometer dispersed in a solution of a solvent comprising n-alkyl acetate having from 3 to 5 carbon atoms in the alkyl group and a film forming polymer consisting essentially of a film forming polymer having a polyvinyl butyral content between about 50 and about 75 mol percent, a polyvinyl alcohol content between about 12 and about 50 mol percent, and a polyvinyl acetate content is between about 0 to 15 mol percent, the photoconductive pigment particles including a mixture of at least two different phthalocyanine pigment particles free of vanadyl phthalocyanine pigment particles, drying the coating to remove substantially all of the alkyl acetate solvent to form a dried charge generation layer comprising between about 50 percent and about 90 percent by weight of the pigment particles based on the total weight of the dried charge generation layer, and forming a charge transport layer.

The disclosures of each of the foregoing patents are hereby incorporated by reference herein in their entireties. The appropriate components and process aspects of the each of the foregoing patents may also be selected for the present compositions and processes in embodiments thereof.

## BACKGROUND

Electrophotographic imaging members, i.e. photoreceptors, typically include a photoconductive layer formed on an electrically conductive substrate. The photoconductive layer is an insulator in the dark so that electric charges are retained on its surface. Upon exposure to light, the charge is dissipated.

Many advanced imaging systems are based on the use of small diameter photoreceptor drums. The use of small diameter drums places a premium on photoreceptor life. A major factor limiting photoreceptor life in copiers and printers, is wear. The use of small diameter drum photoreceptors exacerbates the wear problem because, for example, 3 to 10 revolutions are required to image a single letter size page. Multiple revolutions of a small diameter drum photoreceptor to reproduce a single letter size page can require up to 1 million cycles from the photoreceptor drum to obtain 100,000 prints, a desirable goal for commercial systems.

For low volume copiers and printers, bias charging rolls (BCR) are desirable because little or no ozone is produced during image cycling. However, the micro corona generated by the BCR during charging, damages the photoreceptor, resulting in rapid wear of the imaging surface, e.g., the exposed surface of the charge transport layer. For example, wear rates can be as high as about 16 microns per 100,000 imaging cycles. Similar problems are encountered with bias transfer roll (BTR) systems. One approach to achieving longer photoreceptor drum life is to form a protective overcoat on the imaging surface, e.g. the charge transporting layer of a photoreceptor. This overcoat layer must satisfy many requirements, including transporting holes, resisting image deletion, resisting wear, avoidance of perturbation of underlying layers during coating.

Despite the various approaches that have been taken for forming overcoating layers, there remains a need for improved overcoat layer design, to provide increased wear resistance and resistance to moisture, such as humidity, and the like. A need also exists for improved overcoat layer design, to provide hard yet flexible layers that are more resistant to cracking. For example, the art has previously provided a range of hard overcoating layer materials. However, such overcoat layers are typically prone to cracking, especially

during use, as well as humidity. Both effects tend to reduce the useful life of the photoreceptor, or limit the range of environments and printing apparatus in which the photoreceptor can be used.

## SUMMARY

This disclosure addresses some or all of the above problems, and others, by providing novel, improved photoreceptor overcoat layers. The overcoat layers generally include, as a hole transporting molecule, a hydroxyl-containing hole transport compound. The hydroxyl-containing hole transporting molecule can be mixed with binder materials and suitable crosslinking materials such as crosslinking agents and/or catalysts, to form the overcoating layer.

In an embodiment, the present disclosure provides an electrophotographic imaging member comprising:

- a substrate,
- a charge generating layer,
- a charge transport layer, and

an overcoating layer, said overcoating layer comprising a cured film formed from a film forming resin composition comprising at least a melamine compound, polyol and a charge transport compound, wherein the charge transport compound is represented by:



wherein Q represents a charge transport component, L represents a divalent linkage group, and n represents a number of repeating segments or groups.

The present disclosure also provides electrographic image development devices comprising such electrophotographic imaging members. Also provided are imaging processes using such electrophotographic imaging members.

In another embodiment, the present disclosure provides a process for forming an electrophotographic imaging member comprising:

providing an electrophotographic imaging member comprising a substrate, a charge generating layer, and a charge transport layer, and

forming thereover an overcoating layer comprising a cured film formed from a film forming resin composition comprising at least a melamine compound, a polyol, and a charge transport compound, wherein the charge transport compound is represented by:



wherein Q represents a charge transport component, L represents a divalent linkage group, and n represents a number of repeating segments or groups.

## EMBODIMENTS

Electrophotographic imaging members are known in the art. Electrophotographic imaging members may be prepared by any suitable technique. Typically, a flexible or rigid substrate is provided with an electrically conductive surface. A charge generating layer is then applied to the electrically conductive surface. A charge blocking layer may optionally be applied to the electrically conductive surface prior to the application of a charge generating layer. If desired, an adhesive layer may be utilized between the charge blocking layer and the charge generating layer. Usually the charge generation layer is applied onto the blocking layer and a charge transport layer is formed on the charge generation layer. This structure may have the charge generation layer on top of or below the charge transport layer.

The substrate may be opaque or substantially transparent and may comprise any suitable material having the required mechanical properties. Accordingly, the substrate may comprise a layer of an electrically non-conductive or conductive material such as an inorganic or an organic composition. As electrically non-conducting materials there may be employed various resins known for this purpose including polyesters, polycarbonates, polyamides, polyurethanes, and the like which are flexible as thin webs. An electrically conducting substrate may be any metal, for example, aluminum, nickel, steel, copper, and the like or a polymeric material, as described above, filled with an electrically conducting substance, such as carbon, metallic powder, and the like or an organic electrically conducting material. The electrically insulating or conductive substrate may be in the form of an endless flexible belt, a web, a rigid cylinder, a sheet and the like. The thickness of the substrate layer depends on numerous factors, including strength desired and economical considerations. Thus, for a drum, this layer may be of substantial thickness of, for example, up to many centimeters or of a minimum thickness of less than a millimeter. Similarly, a flexible belt may be of substantial thickness, for example, about 250 micrometers, or of minimum thickness less than 50 micrometers, provided there are no adverse effects on the final electrophotographic device.

In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors. Accordingly, for a flexible photoresponsive imaging device, the thickness of the conductive coating may be about 20 angstroms to about 750 angstroms, such as about 100 angstroms to about 200 angstroms for an optimum combination of electrical conductivity, flexibility and light transmission. The flexible conductive coating may be an electrically conductive metal layer formed, for example, on the substrate by any suitable coating technique, such as a vacuum depositing technique or electrodeposition. Typical metals include aluminum, zirconium, niobium, tantalum, vanadium and hafnium, titanium, nickel, stainless steel, chromium, tungsten, molybdenum, and the like.

An optional hole blocking layer may be applied to the substrate. Any suitable and conventional blocking layer capable of forming an electronic barrier to holes between the adjacent photoconductive layer and the underlying conductive surface of a substrate may be utilized.

An optional adhesive layer may be applied to the hole blocking layer. Any suitable adhesive layer known in the art may be utilized. Typical adhesive layer materials include, for example, polyesters, polyurethanes, and the like. Satisfactory results may be achieved with adhesive layer thickness of about 0.05 micrometer (500 angstroms) to about 0.3 micrometer (3,000 angstroms). Conventional techniques for applying an adhesive layer coating mixture to the charge blocking layer include spraying, dip coating, roll coating, wire wound rod coating, gravure coating, Bird applicator coating, and the like. Drying of the deposited coating may be effected by any suitable conventional technique such as oven drying, infra red radiation drying, air drying and the like.

At least one electrophotographic imaging layer is formed on the adhesive layer, blocking layer or substrate. The electrophotographic imaging layer may be a single layer that performs both charge generating and charge transport functions as is known in the art or it may comprise multiple layers such as a charge generator layer and charge transport layer. Charge generator layers may comprise amorphous films of

selenium and alloys of selenium and arsenic, tellurium, germanium and the like, hydrogenated amorphous silicon and compounds of silicon and germanium, carbon, oxygen, nitrogen and the like fabricated by vacuum evaporation or deposition. The charge generator layers may also comprise inorganic pigments of crystalline selenium and its alloys; Group II-VI compounds; and organic pigments such as quinacridones, polycyclic pigments such as dibromo anthanthrone pigments, perylene and perinone diamines, polynuclear aromatic quinones, azo pigments including bis-, tris- and tetrakis-azos; and the like dispersed in a film forming polymeric binder and fabricated by solvent coating techniques.

Phthalocyanines have been employed as photogenerating materials for use in laser printers utilizing infrared exposure systems. Infrared sensitivity is required for photoreceptors exposed to low cost semiconductor laser diode light exposure devices. The absorption spectrum and photosensitivity of the phthalocyanines depend on the central metal atom of the compound. Many metal phthalocyanines have been reported and include, oxyvanadium phthalocyanine, chloroaluminum phthalocyanine, copper phthalocyanine, oxytitanium phthalocyanine, chlorogallium phthalocyanine, hydroxygallium phthalocyanine, magnesium phthalocyanine and metal-free phthalocyanine. The phthalocyanines exist in many crystal forms which have a strong influence on photogeneration.

Any suitable polymeric film forming binder material may be employed as the matrix in the charge generating (photogenerating) binder layer. Typical polymeric film forming materials include those described, for example, in U.S. Pat. No. 3,121,006, the entire disclosure of which is incorporated herein by reference. Thus, typical organic polymeric film forming binders include thermoplastic and thermosetting resins such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrenebutadiene copolymers, vinylidenechloride-vinylchloride copolymers, vinylacetate-vinylidenechloride copolymers, styrene-alkyd resins, polyvinylcarbazole, and the like. These polymers may be block, random or alternating copolymers.

The photogenerating composition or pigment is present in the resinous binder composition in various amounts. Generally, however, from about 5 percent by volume to about 90 percent by volume of the photogenerating pigment is dispersed in about 10 percent by volume to about 95 percent by volume of the resinous binder, such as from about 20 percent by volume to about 30 percent by volume of the photogenerating pigment dispersed in about 70 percent by volume to about 80 percent by volume of the resinous binder composition. In one embodiment about 8 percent by volume of the photogenerating pigment is dispersed in about 92 percent by volume of the resinous binder composition. The photogenerator layers can also be fabricated by vacuum sublimation in which case there is no binder.

Any suitable and conventional technique may be utilized to mix and thereafter apply the photogenerating layer coating mixture. Typical application techniques include spraying, dip coating, roll coating, wire wound rod coating, vacuum sublimation and the like. For some applications, the generator layer may be fabricated in a dot or line pattern. Removing of

the solvent of a solvent coated layer may be effected by any suitable conventional technique such as oven drying, infrared radiation drying, air drying and the like.

The charge transport layer may comprise a charge transporting small molecule dissolved or molecularly dispersed in a film forming electrically inert polymer such as a polycarbonate. The term "dissolved" as employed herein is defined herein as forming a solution in which the small molecule is dissolved in the polymer to form a homogeneous phase. The expression "molecularly dispersed" is used herein as defined as a charge transporting small molecule dispersed in the polymer, the small molecules being dispersed in the polymer on a molecular scale. Any suitable charge transporting or electrically active small molecule may be employed in the charge transport layer. The expression charge transporting "small molecule" is defined herein as a monomer that allows the free charge photogenerated in the transport layer to be transported across the transport layer. Typical charge transporting small molecules include, for example, pyrazolines such as 1-phenyl-3-(4'-diethylamino styryl)-5-(4"-diethylamino phenyl) pyrazoline, diamines such as N,N'-diphenyl-N,N'-bis(3-methylphenyl)-(1,1'-biphenyl)-4,4'-diamine, hydrazones such as N-phenyl-N-methyl-3-(9-ethyl)carbazyl hydrazone and 4-diethyl amino benzaldehyde-1,2-diphenyl hydrazone, and oxadiazoles such as 2,5-bis(4-N,N'-diethylaminophenyl)-1,2,4-oxadiazole, stilbenes and the like. As indicated above, suitable electrically active small molecule charge transporting compounds are dissolved or molecularly dispersed in electrically inactive polymeric film forming materials. A small molecule charge transporting compound that permits injection of holes from the pigment into the charge generating layer with high efficiency and transports them across the charge transport layer with very short transit times is N,N'-diphenyl-N,N'-bis(3-methylphenyl)-(1,1'-biphenyl)-4,4'-diamine. If desired, the charge transport material in the charge transport layer may comprise a polymeric charge transport material or a combination of a small molecule charge transport material and a polymeric charge transport material.

Any suitable electrically inactive resin binder insoluble in the alcohol solvent used to apply the overcoat layer may be employed in the charge transport layer. Typical inactive resin binders include polycarbonate resin, polyester, polyarylate, polysulfone, and the like. Molecular weights can vary, for example, from about 20,000 to about 150,000. Exemplary binders include polycarbonates such as poly(4,4'-isopropylidene-diphenylene)carbonate (also referred to as bisphenol-A-polycarbonate, poly(4,4'-cyclohexylidinediphenylene) carbonate (referred to as bisphenol-Z polycarbonate), poly(4,4'-isopropylidene-3,3'-dimethyl-diphenyl)carbonate (also referred to as bisphenol-C-polycarbonate) and the like. Any suitable charge transporting polymer may also be utilized in the charge transporting layer. The charge transporting polymer should be insoluble in any solvent employed to apply the subsequent overcoat layer described below, such as an alcohol solvent. These electrically active charge transporting polymeric materials should be capable of supporting the injection of photogenerated holes from the charge generation material and be incapable of allowing the transport of these holes therethrough.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like.

Generally, the thickness of the charge transport layer is between about 10 and about 50 micrometers, but thicknesses outside this range can also be used. The hole transport layer should be an insulator to the extent that the electrostatic charge placed on the hole transport layer is not conducted in the absence of illumination at a rate sufficient to prevent formation and retention of an electrostatic latent image thereon. In general, the ratio of the thickness of the hole transport layer to the charge generator layers is desirably maintained from about 2:1 to 200:1 and in some instances as great as 400:1. The charge transport layer, is substantially non-absorbing to visible light or radiation in the region of intended use but is electrically "active" in that it allows the injection of photogenerated holes from the photoconductive layer, i.e., charge generation layer, and allows these holes to be transported through itself to selectively discharge a surface charge on the surface of the active layer.

To improve photoreceptor wear resistance, a protective overcoat layer is provided over the charge transport layer. The overcoat layer generally includes a film-forming resin composition comprising at least a melamine compound, a polyol and a hole transporting molecule. The overcoating layer can be formed, for example, from a solution or other suitable mixture of the film-forming resin composition, and other optional additives. For example, the overcoating layer can be formed from a solution comprising the film forming resin composition of at least a melamine compound or resin, a polyol and a charge transport compound in a solvent. In embodiments, the film forming resin composition can include from about 5 to about 80 percent by weight of charge transport compound, from about 5 to about 90 percent by weight of polyol polymer and from about 70 to about 5 percent by weight of melamine compound, although other amounts can be used.

A polyol is generally defined as a compound or polymer containing multiple pendent hydroxyl groups. Examples of such polyol polymers include an aliphatic polyester polyol, an aromatic polyester polyol, an acrylated polyol, an aliphatic polyether polyol, an aromatic polyether polyol, a (polystyrene-co-polyacrylate) polyol, polyvinyl butylral, poly(2-hydroxyethyl methacrylate) and the like. For example, in embodiments, the polyol polymer can be a polyester polyol or acrylated polyol, such as a highly branched polyester polyol or acrylated polyol. The term "highly branched" refers, for example, to a prepolymer synthesized using a significant amount of trifunctional alcohols, such as triols, to form a polymer having a significant number of branches off of the main polymer chain. This is distinguished from a linear prepolymer that contains only difunctional monomers, and thus little or no branches off of the main polymer chain. The term "polyester polyol" refers, for example, to such compounds that include multiple ester groups as well as multiple alcohol (hydroxyl) groups in the molecule, and which can include other groups such as, for example, ether groups and the like. In embodiments, the polyester polyol can thus include ether groups, or can be free of ether groups. Likewise, the term "acrylated polyol" refers, for example, to such compounds that include multiple ether groups as well as multiple alcohol (hydroxyl) groups in the molecule, and which can include acrylate groups such as, for example, methacrylate groups and the like.

Examples of such suitable polyester polyols include, for example, polyester polyols formed from the reaction of a polycarboxylic acid such as a dicarboxylic acid or a tricarboxylic acid (including acid anhydrides) with a polyol such as a diol or a triol. In embodiments, the number of ester and alcohol groups, and the relative amount and type of polyacid

and polyol, should be selected such that the resulting polyester polyol compound retains a number of free hydroxyl groups, which can be used for subsequent crosslinking of the material in forming the overcoating layer binder material. For example, suitable polycarboxylic acids include, but are not limited to, adipic acid (COOH[CH<sub>2</sub>]<sub>4</sub>COOH), pimelic acid (COOH[CH<sub>2</sub>]<sub>5</sub>COOH), suberic acid (COOH[CH<sub>2</sub>]<sub>6</sub>COOH), azelaic acid (COOH[CH<sub>2</sub>]<sub>7</sub>COOH), sebasic acid (COOH[CH<sub>2</sub>]<sub>8</sub>COOH), and the like. Suitable polyols include, but are not limited to, difunctional materials such as glycols or trifunctional alcohols such as triols and the like, including propanediols (HO[CH<sub>2</sub>]<sub>3</sub>OH), butanediols (HO[CH<sub>2</sub>]<sub>4</sub>OH), hexanediols (HO[CH<sub>2</sub>]<sub>6</sub>OH), glycerine (HOCH<sub>2</sub>CHOHCH<sub>2</sub>OH), 1,2,6-Hexane triol (HOCH<sub>2</sub>CHOH[CH<sub>2</sub>]<sub>4</sub>OH), and the like.

In embodiments, the suitable polyester polyols are reaction products of polycarboxylic acids and polyols and can be represented by the following formula (1):



where Ra and Rc independently represent linear alkyl groups or branched alkyl groups derived from the polyols, the alkyl groups having from 1 to about 20 carbon atoms; Rb and Rd independently represent alkyl or aryl groups derived from the polycarboxylic acids, the alkyl groups having from 1 to about 20 carbon atoms; the aryl groups having from 6 to about 60 carbon atoms and m, n, p, and q represent mole fractions of from 0 to 1, such that n+m+p+q=1.

Specific commercially available examples of such suitable polyester polyols include, for example: the DESMOPHEN® series of products available from Bayer Chemical, including the DESMOPHEN® 800, 1110, 1112, 1145, 1150, 1240, 1262, 1381, 1400, 1470, 1630, 2060, 2061, 2062, 3060, 4027, 4028, 404, 4059, 5027, 5028, 5029, 5031, 5035, and 5036 products; the SOVERMOL® series of products available from Cognis, including the SOVERMOL® 750, 805, 815, 908, 910, and 913 products; and the HYDAGEN® series of products available from Cognis, including the HYDAGEN® HSP product; and mixtures thereof. Particularly preferred in embodiments are DESMOPHEN® 800 and SOVERMOL® 750, or mixtures thereof. DESMOPHEN® 800 is a highly branched polyester bearing hydroxyl groups, having an acid value of  $\leq 4$  mg KOH/g, a hydroxyl content of about  $8.6 \pm 0.3\%$ , and an equivalent weight of about 200. DESMOPHEN® 800 corresponds to the above formula (1) where the polymer contains 50 parts adipic acid, 10 parts phthalic anhydride, and 40 parts 1,2,6-hexanetriol, where Rb=—[CH<sub>2</sub>]<sub>4</sub>—, n=0.5, Rd=—1,2-C<sub>6</sub>H<sub>4</sub>—, q=0.1, Ra=Rc=—CH<sub>2</sub>[CHO—][CH<sub>2</sub>]<sub>4</sub>—, and m+p=0.4. DESMOPHEN® 1100 corresponds to the above formula (1) where the polymer contains 60 parts adipic acid, 40 parts 1,2,6-hexanetriol, and 60 parts 1,4-butanediol, where Rb=Rd=—[CH<sub>2</sub>]<sub>4</sub>—, n+q=0.375, Ra=—CH<sub>2</sub>[CHO—][CH<sub>2</sub>]<sub>4</sub>—, m=0.25, Rc=—[CH<sub>2</sub>]<sub>4</sub>—, and p=0.375. SOVERMOL® 750 is a branched polyether/polyester/polyol having an acid value of  $\leq 2$  mg KOH/g, and a hydroxyl value of 300-330 mg KOH/g.

In other embodiments, the polyol can be an acrylated polyol. Suitable acrylated polyols can be, for example, the reaction products of propylene oxide modified with ethylene oxide, glycols, triglycerol and the like. These polyols are further reacted with substituted acrylic acids, alcohol containing acrylates, substituted acryloyl chlorides, and the like, forming terminal acrylate groups. Such acrylated polyols can be represented by the following formula (2):

## 11



where  $R_t$  represent  $CH_2CR_1CO_2$ — where  $R_1$  is an alkyl group of from 1 to about 20 carbon atoms or more such as methyl, ethyl, and the like and where  $t$  represents mole fractions of acrylated sites from 0 to 1.  $R_a$  and  $R_c$ , independently represent linear alkyl/alkoxy groups or branched alkyl/alkoxy groups derived from the polyols, the alkyl/alkoxy groups having from 1 to about 20 carbon atoms;  $R_b$  and  $R_d$  independently represent alkyl/alkoxy groups, the alkyl/alkoxy groups having from 1 to about 20 carbon atoms; and  $m$ ,  $n$ ,  $p$ , and  $q$  represent mole fractions of from 0 to 1, such that  $n+m+p+q=1$ . In formula (2), the notation “[ $R_t-CH_2$ ] $_t$ —” indicates that the acrylate groups react with some of the hydroxyl groups in the main chain or branches of the polyol component.

In other embodiments, the polyol can be a polyether polyol. Suitable polyether polyols can be, for example, the reaction products of propylene oxide modified with ethylene oxide, glycols, triglycerol and the like. Such polyols can be represented by the following formula (3):



where  $R_a$  and  $R_c$  independently represent linear alkyl/alkoxy groups or branched alkyl/alkoxy groups derived from the polyols, the alkyl/alkoxy groups having from 1 to about 20 carbon atoms;  $R_b$  and  $R_d$  independently represent alkyl/alkoxy groups, the alkyl/alkoxy groups having from 1 to about 20 carbon atoms; aryl groups having from 6 to about 60 carbon atoms and  $m$ ,  $n$ ,  $p$ , and  $q$  represent mole fractions of from 0 to 1, such that  $n+m+p+q=1$ . Typical examples of aromatic polyether polyols include bisphenol A ethoxylate, bisphenol A propoxylate, bisphenol A propoxylate/ethoxylate, poly(bisphenol A-co-epichlorohydrin), and the like.

In still other embodiments, the overcoating layer may contain any suitable film-forming resin, including any of those described above for use in the other layers of the imaging member. In these embodiments, the film-forming resin can be electrically insulating, semi-conductive, or conductive, and can be hole transporting or not hole transporting. Thus, for example, suitable film-forming resins can be selected from thermoplastic and thermosetting resins such as polycarbonates, polyesters, polyamides, polyurethanes, polystyrenes, polyarylethers, polyarylsulfones, polysulfones, polyethersulfones, polyphenylene sulfides, polyvinyl acetate, polyacrylates, polyvinyl acetals, polyamides, polyimides, amino resins, phenylene oxide resins, phenoxy resins, epoxy resins, phenolic resins, polystyrene and acrylonitrile copolymers, vinyl acetate copolymers, acrylate copolymers, alkyd resins, styrenebutadiene copolymers, styrene-alkyd resins, polyvinylcarbazole, and the like. These polymers may be block, random or alternating copolymers.

In forming the binder material for the overcoating layer, any suitable crosslinking agents, catalysts, and the like can be included in known amounts for known purposes. For example, in embodiments a crosslinking agent or accelerator, such as a melamine crosslinking agent or accelerator, can be included with the polyester polyol or acrylated polyol for forming the overcoating layer. Incorporation of a crosslinking agent or accelerator provides reaction sites to interact with the polyester polyol or acrylated polyol, to provide a branched, crosslinked structure. When so incorporated, any suitable

## 12

crosslinking agent or accelerator can be used, including, for example, trioxane, melamine compounds, and mixtures thereof.

Where melamine compounds or resins are used in the overcoating layer, any suitable melamine compound can be used. The melamine compounds can be suitably functionalized to be, for example, melamine formaldehyde, alkylated melamine-formaldehyde compounds or resins, such as where the alkyl group has from about one to about ten or from one to about four carbon atoms, methoxymethylated melamine compounds, such as glycouril-formaldehyde and benzoguanamine-formaldehyde, and the like. An example of a suitable methoxymethylated melamine compound is Cymel 303 (available from Cytec Industries), which is a methoxymethylated melamine compound with the formula  $(CH_3OCH_2)_6N_3C_3N_3$  and the following structure:



Typical melamine resins include poly(melamine-formaldehyde), alkylated poly(melamine-formaldehyde) such as methylated poly(melamine-formaldehyde), butylated poly(melamine-formaldehyde), isobutylated poly(melamine-formaldehyde), methylated/butylated poly(melamine-formaldehyde) and the like.

Crosslinking is generally accomplished by heating in the presence of a catalyst. Thus, the solution of the film forming composition can also include a suitable catalyst. Any suitable catalyst may be employed. Typical catalysts include, for example, oxalic acid, maleic acid, carbollylic acid, ascorbic acid, malonic acid, succinic acid, tartaric acid, citric acid, p-toluenesulfonic acid, methanesulfonic acid, and the like and mixtures thereof.

If desired or necessary, a blocking agent can also be included. A blocking agent can be used to “tie up” or block the acid effect to provide solution stability until the acid catalyst function is desired. Thus, for example, the blocking agent can block the acid effect until the solution temperature is raised above a threshold temperature. For example, some blocking agents can be used to block the acid effect until the solution temperature is raised above about 100° C. At that time, the blocking agent dissociates from the acid and vaporizes. The unassociated acid is then free to catalyze the polymerization. Examples of such suitable blocking agents include, but are not limited to, pyridine and commercial acid solutions containing blocking agents such as Cycat 4040 available from Cytec Ind.

The temperature used for crosslinking varies with the specific catalyst and heating time utilized and the degree of crosslinking desired. Generally, the degree of crosslinking selected depends upon the desired flexibility of the final photoreceptor. For example, complete crosslinking may be used for rigid drum or plate photoreceptors. However, partial crosslinking can be beneficial for flexible photoreceptors having, for example, web or belt configurations. The degree of crosslinking can be controlled by the relative amount of catalyst employed. The amount of catalyst to achieve a desired degree of crosslinking will vary depending upon the

## 13

specific coating solution materials, such as polyol, catalyst, temperature and time used for the reaction. In embodiments, the polyol is cross linked at a temperature of about 100° C. to about 150° C. A typical cross linking temperature used for polyols with p-toluenesulfonic acid as a catalyst is less than about 140° C. for about 40 minutes. A typical concentration of acid catalyst is about 0.01 to about 5.0 weight percent based on the weight of polyol. After crosslinking, the overcoating should be substantially insoluble in the solvent in which it was soluble prior to crosslinking. Thus, no overcoating material will be removed when rubbed with a cloth soaked in the solvent. Crosslinking results in the development of a three dimensional network which restrains the transport molecule in the crosslinked polymer network.

Any suitable alcohol solvent may be employed for the film forming polymers. Typical alcohol solvents include, for example, butanol, propanol, methanol, 1-methoxy-2-propanol, and the like and mixtures thereof. Other suitable solvents that can be used in forming the overcoating layer solution include, for example, tetrahydrofuran, monochlorobenzene, and mixtures thereof. These solvents can be used in addition to, or in place of, the above alcohol solvents, or they can be omitted entirely. However, in some embodiments, higher boiling alcohol solvents are avoided, as they can interfere with the desired cross-linking reaction.

Any suitable hole transport material may be utilized in the overcoating layer. However, to provide one or more desired benefits including resistance to cracking, desired mechanical properties, resistance to image deletion, and the like, embodiments include a hydroxyl-containing hole transport compound as a hole transporting molecule.

Exemplary hydroxyl-containing hole transport compounds include those of the following formula:



wherein Q represents a charge transport component, L represents a divalent linkage group, and n represents a number of repeating segments or groups such as from 1 to about 8.

Any suitable charge transport compound can be used as the moiety Q. For example, suitable charge transport compounds include amines, such as tertiary arylamines, pyrazolines, hydrazones, oxazoles, stilbenes, and mixtures thereof.

More specifically, in embodiments, Q is represented by the following general formula



wherein Ar<sup>1</sup>, Ar<sup>2</sup>, Ar<sup>3</sup>, Ar<sup>4</sup> and Ar<sup>5</sup> each independently represents a substituted or unsubstituted aryl group, or Ar<sup>5</sup> independently represents a substituted or unsubstituted arylene group, and k represents 0 or 1, wherein at least one of Ar<sup>1</sup>, Ar<sup>2</sup>, Ar<sup>3</sup> and Ar<sup>4</sup> is connected to the linkage group L.

For example, in embodiments, Ar<sup>1</sup>, Ar<sup>2</sup>, Ar<sup>3</sup>, Ar<sup>4</sup> and Ar<sup>5</sup> each independently represents a substituted or unsubstituted aryl group, such as



## 14



5

where R is selected from the group consisting of an alkyl group having 1 to about 10 carbon atoms, such as —CH<sub>3</sub>, —C<sub>2</sub>H<sub>5</sub>, —C<sub>3</sub>H<sub>7</sub>, and —C<sub>4</sub>H<sub>9</sub>, or Ar<sup>5</sup> independently represents a substituted or unsubstituted arylene group, such as



15

where R is selected from the group consisting of an alkyl group having 1 to about 10 carbon atoms, such as —CH<sub>3</sub>, —C<sub>2</sub>H<sub>5</sub>, —C<sub>3</sub>H<sub>7</sub>, and —C<sub>4</sub>H<sub>9</sub>. Other suitable groups for Ar<sup>5</sup>, when k is greater than 0, include:



20

where n is 0 or 1, Ar is any of the group defined above for Ar<sup>1</sup>, Ar<sup>2</sup>, Ar<sup>3</sup>, Ar<sup>4</sup> and Ar<sup>5</sup>, and X is selected from the group consisting of:



25

where s is 0, 1 or 2.

In embodiments, more specifically, Q is a compound selected from the following:

15



5

10

15

20

25

30

35

40

45

16  
-continued

and mixtures thereof, wherein R<sub>1</sub> to R<sub>19</sub> are independently selected from the group comprised of a hydrogen atom, an alkyl such as having from 1 to about 20 carbon atoms, a cyclic alkyl such as having from 4 to about 20 carbon atoms, an alkoxy group such as having from 1 to about 20 carbon atoms, and halogen, and subscripts a to p each independently represents an integer of 1 or 2. In other embodiments, the charge transport compound Q is selected from the following:



50

55

60

65



and mixtures thereof.

In the above exemplary hydroxyl-containing hole transport compound, L represents a divalent linkage group. In embodiments, the divalent linkage L can be a divalent hydrocarbyl group such as containing from 1 to about 20 carbon atoms or from 1 to about 15 carbon atoms, optionally further containing a heteroatom such as oxygen, sulfur, silicon, and nitrogen. Specific examples of suitable divalent linkage groups L include alkyl groups  $-(\text{CH}_2)_y-$ , where y is an integer from 1 to about 15 or from 1 to about 10, such as methylene or ethylene,



and combination thereof.

In the above exemplary hydroxyl-containing hole transport compound, n represents an integer of 1 to about 8. In embodiments, n is 1 to about 3 or 1 to about 4, such as 1, 2, 3, or 4. For example, when n=2, the compound is represented as a dihydroxylalkyl arylamine compound hole transporting molecule.

If desired, the hydroxyl-containing hole transport compound, such as a hydroxylalkyl arylamine, can be used in combinations of two or more, such as two, three, four or more different hydroxyl-containing hole transport compounds, or one or more hydroxyl-containing hole transport compounds can be used in combination with one or more other types of hole transporting molecules.

Typically hydroxyl-containing hole transport compounds can be readily prepared by known processes. For example, the exemplary compound N,N-bis(4-hydroxymethylphenyl)-3,4-dimethylphenylamine can be prepared from a halogenated dimethylbenzene and a diphenylamine according to the following reaction scheme:

45 N,N-bisphenyl-3,4-dimethylphenylamine can be prepared by known Ulmann condensation process. The bisformalation of N,N-bisphenyl-3,4-dimethylphenylamine affords the bisformalated arylamine intermediate. Reduction of the aldehydes leads to the final product, N,N-bis(4-hydroxymethylphenyl)-3,4-dimethylphenylamine. Other hydroxyl-containing hole transport compounds can be readily made by modification of the above reaction scheme.

50 The thickness of the continuous overcoat layer selected depends upon the abrasiveness of the charging (such as bias charging roll), cleaning (such as blade or web), development (such as brush), transfer (such as bias transfer roll), and the like in the system employed and can range from about 1 or 55 about 2 microns up to about 10 or about 15 microns or more. A thickness of about 1 micrometer to about 5 micrometers is desired, in embodiments. Typical application techniques include spraying, dip coating, roll coating, wire wound rod coating, and the like. Drying of the deposited coating may be effected by any suitable conventional technique such as oven drying, infrared radiation drying, air drying and the like. The dried overcoating of this disclosure should transport holes during imaging and should not have too high a free carrier concentration. Free carrier concentration in the overcoat increases the dark decay. In embodiments, the dark decay of the overcoated layer should be about the same as that of the unovercoated device.

19

In the dried overcoating layer, the composition can include from about 10 to about 90 percent by weight film-forming binder, and from about 90 to about 10 percent by weight hole transporting molecule. For example, in embodiments, the hole transporting molecule can be incorporated into the overcoating layer in an amount of from about 20 to about 70 percent by weight, such as about 33 percent by weight. As desired, the overcoating layer can also include other materials, such as conductive fillers, abrasion resistant fillers, and the like, in any suitable and known amounts.

Advantages provided by the present disclosure include, in embodiments, overcoating layers that robust and provide desirable electrical and mechanical properties. Some overcoat layers possess these properties, but can exhibit undesired image deletion, an image defect that tends to occur after extended use of the coated imaging members. In embodiments, the overcoat layer exhibits excellent resistance to abrasion, resistance to scratching and cracking without adversely affecting electrical performance of photoreceptors. Therefore, the coated photoreceptor devices demonstrate extended service life while maintaining desirable image quality.

Also, included within the scope of the present disclosure are methods of imaging and printing with the imaging members illustrated herein. These methods generally involve the formation of an electrostatic latent image on the imaging member; followed by developing the image with a toner composition comprised, for example, of thermoplastic resin, colorant, such as pigment, charge additive, and surface additives, reference U.S. Pat. Nos. 4,560,635, 4,298,697 and 4,338,390, the disclosures of which are totally incorporated herein by reference; subsequently transferring the image to a suitable substrate; and permanently affixing the image thereto. In those environments wherein the device is to be used in a printing mode, the imaging method involves the same steps with the exception that the exposure step can be accomplished with a laser device or image bar.

An example is set forth hereinbelow and is illustrative of different compositions and conditions that can be utilized in practicing the disclosure. All proportions are by weight unless otherwise indicated. It will be apparent, however, that the disclosure can be practiced with many types of compositions and can have many different uses in accordance with the disclosure above and as pointed out hereinafter.

## EXAMPLES

### Example 1

#### Preparation of Hydroxyl-Containing Hole Transport Compound

The hydroxyl-containing hole transport compound N,N-bis(4-hydroxymethylphenyl)-3,4-dimethylphenylamine was prepared as follows:



20

-continued



N,N-bisphenyl-3,4-dimethylphenylamine was prepared by known Ulmann condensation process.

A mixture of N,N-bisphenyl-3,4-dimethylphenylamine (162 g), zinc chloride (80.76 g), DMF (129.94 g) and Isopar L (222 g) was charged in a 3-L RB (round bottom) flask. Phosphorus oxychloride (272.62 g) was added drop-wise into the reaction mixture under Argon while stirring. The reaction mixture was heated to 120° C. and this temperature was maintained for 12 hours. About 500 g of N,N-dimethylformamide were then added to the resulting mixture. The reaction mixture was cooled to about 50° C., and poured into 2.5 L of water with mechanical stirring. The resulting precipitates were collected by filtration and washed with water (2L) twice, and then refluxed in toluene with about 150 g of an acidic clay. After the clay treatment, the toluene solution was collected and stirred with about 100 g of silica gel at room temperature, about 23 to about 25° C. for 1 hour. After removal of toluene, the product was collected and dried at 40° C. for 1 hour. The yield of the bisformalation was 141.3 g (71%).

The bisformalated arylamine product obtained from the above preparation (139 g) was mixed with 700 mL of ethanol in a 1-L 3-neck round-bottomed flask equipped with a magnetic stirrer, and an argon introduction tube. To the suspension resulting was added 0.1 gram of NaOH and 15.96 g of NaBH<sub>4</sub>. The reaction was conducted for 1 hour at room temperature (25° C.). The solution obtained was poured into 2.5 L of water and the resulting pale yellow solids were collected by filtration, and then washed with 2 L of water. Drying at 40° C. overnight, 18 to 20 hours generated 137 g of crude product in 97.4% yield. Recrystallization in toluene (600 mL) and drying at room temperature under high vacuum yielded 132.8 g of pure product (94.4%). The structure of the desired prod-

21

uct N,N-bis(4-hydroxymethylphenyl)-3,4-dimethylphenylamine was confirmed with  $^1\text{H}$  NMR spectrum.

## Example 2

## Preparation of Overcoating Composition

A coating composition was formed containing 1 gram DESMOPHEN® 800 polyester polyol, 0.6 gram Cymel 1130, 0.8 gram hole transporting molecule N,N-bis(4-hydroxymethylphenyl)-3,4-dimethylphenylamine of Example 1, 7.2 grams 1-methoxy-2-propanol (Dowanol PM), and 0.2 grams of p-toluenesulfonic acid/pyridine (8% acid/4% pyridine in 1-methoxy-2-propanol) as catalyst. The components were mixed and shaken at room temperature (about 20° C. to about 25° C.) until all of the components were dissolved.

## Comparative Example 1

## Preparation of Overcoating Composition

A coating composition was formed as in Example 2, except that the 0.8 gram hole transporting molecule N,N-bis(4-hydroxymethylphenyl)-3,4-dimethylphenylamine was replaced by 0.6 gram hole transporting molecule N,N'-diphenyl-N,N'-bis(3-hydroxyphenyl)-[1,1'-biphenyl]-4,4'-diamine.

## Example 3

## Preparation of Overcoated Imaging Member

An overcoated imaging member sheet or belt is formed using the coating composition of Example 2. In particular, an electrophotographic imaging member web stock is prepared by providing a 0.02 micrometer thick titanium layer coated on a biaxially oriented polyethylene naphthalate substrate (Kadalex, available from ICI Americas, Inc.) having a thickness of 3.5 mils (89 micrometers) and applying thereto, using a gravure coating technique and a solution containing 10 grams gamma aminopropyltriethoxy silane, 10.1 grams distilled water, 3 grams acetic acid, 684.8 grams of 200 proof denatured alcohol and 200 grams heptane. This layer is then allowed to dry for 5 minutes at 135° C. in a forced air oven. The resulting blocking layer has an average dry thickness of 0.05 micrometer measured with an ellipsometer.

An adhesive interface layer is then prepared by applying with extrusion process to the blocking layer a wet coating containing 5 percent by weight based on the total weight of the solution of polyester adhesive (Mor-Ester 49,000, available from Morton International, Inc.) in a 70:30 volume ratio mixture of tetrahydrofuran:cyclohexanone. The adhesive interface layer is allowed to dry for 5 minutes at 135° C. in a forced air oven. The resulting adhesive interface layer has a dry thickness of 0.065 micrometer.

The adhesive interface layer is thereafter coated with a photogenerating layer. The photogenerating layer dispersion is prepared by introducing 0.45 grams of Iupilon 200 (PC-Z 200) available from Mitsubishi Gas Chemical Corp and 50 ml of tetrahydrofuran into a 4 oz. glass bottle. To this solution is added 2.4 grams of hydroxygallium phthalocyanine and 300 grams of  $\frac{1}{8}$  inch (3.2 millimeter) diameter stainless steel shot. This mixture is then placed on a ball mill for 20 to 24 hours. Subsequently, 2.25 grams of PC-Z 200 is dissolved in 46.1 gm of tetrahydrofuran, then added to this OHGaPc slurry. This slurry is then placed on a shaker for 10 minutes. The resulting slurry is, thereafter, coated onto the adhesive interface by an extrusion application process to form a layer having a wet

22

thickness of 0.25 mil. However, a strip about 10 mm wide along one edge of the substrate web bearing the blocking layer and the adhesive layer is deliberately left uncoated by any of the photogenerating layer material to facilitate adequate electrical contact by the ground strip layer that is applied later. This photogenerating layer is dried at 135° C. for 5 minutes in a forced air oven to form a dry thickness photogenerating layer having a thickness of 0.4 micrometer layer.

10 This coated imaging member web is simultaneously overcoated with a charge transport layer and a ground strip layer using extrusion co-coating process. The charge transport layer is prepared by introducing into an amber glass bottle a weight ratio of 1:1 N,N'-diphenyl-N,N'-bis(3-methylphenyl)-1,1'-biphenyl-4,4'-diamine, and Makrolon 5705, a polycarbonate resin having a weight average molecular weight of about 120,000 commercially available from Bayer A.G. The resulting mixture is dissolved to give a 15 percent by weight solid in 85 percent by weight methylene chloride. This solution is applied onto the photogenerator layer to form a coating which upon drying has a thickness of 29 micrometers.

15 The approximately 10 mm wide strip of the adhesive layer left uncoated by the photogenerator layer is coated over with a ground strip layer during the co-coating process. This ground strip layer, after drying along with the co-coated charge transport layer at 135° C. in the forced air oven for minutes, has a dried thickness of about 19 micrometers. This ground strip is electrically grounded, by conventional means such as a carbon brush contact means during conventional xerographic imaging process.

20 An anticurl coating is prepared by combining 8.82 grams of polycarbonate resin (Makrolon 5705, available from Bayer AG), 0.72 gram of polyester resin (Vitel PE-200, available from Goodyear Tire and Rubber Company) and 90.1 grams of 25 methylene chloride in a glass container to form a coating solution containing 8.9 percent solids. The container is covered tightly and placed on a roll mill for about 24 hours until the polycarbonate and polyester are dissolved in the methylene chloride to form the anticurl coating solution. The anti-30 curl coating solution is then applied to the rear surface (side opposite the photogenerator layer and charge transport layer) of the imaging member web stock, again by extrusion coating process, and dried at 135° C. for about 5 minutes in the forced air oven to produce a dried film thickness of about 17 40 micrometers.

45 The sheet is overcoated with the overcoat layer composition of Example 2. The coating composition is filtered through a 0.45 micron filter, and is applied using a 0.125 mil Bird bar applicator and dried at 125° C. for 4 minutes. The 50 result is an imaging member having an overcoating layer thickness of 3 microns.

## Comparative Example 2

## Preparation of Overcoated Imaging Member

An imaging member is made in the same manner as in Example 3, except that the overcoating layer is prepared using the composition of Comparative Example 1.

## Comparative Example 3

## Preparation of Control Imaging Member

55 An imaging member was made in the same manner as in Example 3, except that the overcoating layer is omitted. This 60 imaging member is used as a control.

23

## Example 4

## Testing of Imaging Members

The imaging members of Example 3 and Comparative Examples 2 and 3 are tested for their electrostatographic sensitivity and cycling stability in a scanner. The scanner is known in the industry and equipped with means to rotate the drum while it is electrically charged and discharged. The charge on the sample is monitored through use of electrostatic probes placed at precise positions around the circumference of the device. The samples in this Example are charged to a negative potential of 500 Volts. As the device rotates, the initial charging potential is measured by voltage probe 1. The sample is then exposed to monochromatic radiation of known intensity, and the surface potential measured by voltage probes 2 and 3. Finally, the sample is exposed to an erase lamp of appropriate intensity and wavelength and any residual potential is measured by voltage probe 4. The process is repeated under the control of the scanner's computer, and the data is stored in the computer. The PIDC (photo induced discharge curve) is obtained by plotting the potentials at voltage probes 2 and 3 as a function of the light energy.

The results show comparable PIDC curves for all three samples. This indicates that the overcoating layer provides comparable electrical results to the control imaging member without an overcoating layer.

Image deletion tests are also conducted on the imaging members of Example 3 and Comparative Examples 2 and 3. The test is conducted by laminating a strip (about 8 inch×1.5 inch) of the overcoated imaging member of Example 3 and a strip (about 8 inch×1.5 inch) of the reference imaging member of Comparative Example 3 on the photoreceptor drum of a Xerox DocuCentre 12 office machine using conductive adhesive tape. The tape is used to hold the laminated strips in place and also to provide electrical contact between the conductive layer in each of the two strips and the drum metal base. The drum configuration is then mounted in an axial scanner equipped with a scorotron charging element and an erase laser bar. The scanner allows for the repetitive charging and discharging of the drum configuration by means of rotating the drum at a rate of 150 cycles per minute between the scorotron (where the drum surface in close proximity to the scorotron gets charged to a potential of about 750 volts) and discharged by means of exposure to the laser beam. The cycling is carried in ambient conditions for a total of about 170,000 cycles. Following cycling, the drum configurations are then removed from the axial scanner and mounted in a Xerox DocuCentre 12 office machine. The machine is then used to print a variable-width multiple-lined print pattern on 11"×17" standard white paper. The printed pattern is then examined visually on the paper for line blurriness. A comparison between print patterns produced by drum areas laminated by a strip of the overcoated imaging member of Example 3 and a strip of the reference imaging member of Comparative Example 3 is then done.

The testing showed that the imaging member of Example 3 was very resistant to image deletion, exhibiting stable performance over 170,000 cycles. In contrast, the imaging members of Comparative Examples 2 and 3 showed poor image deletion resistance. In particular, the control imaging member of Comparative Example 3 exhibited image deletion after about 50,000 cycles, and the imaging member of Comparative Example 2 exhibited image deletion after about 20,000 cycles.

It will be appreciated that various of the above-disclosed and other features and functions, or alternatives thereof,

24

maybe desirably combined into many other different systems or applications. Also that various presently unforeseen or unanticipated alternatives, modifications, variations or improvements therein may be subsequently made by those skilled in the art which are also intended to be encompassed by the following claims.

What is claimed is:

1. An electrophotographic imaging member comprising:  
a substrate,  
a charge generating layer,  
a charge transport layer, and  
an overcoating layer, said overcoating layer comprising a cured film formed from a film forming resin composition comprising at least a melamine compound, a polyol and a charge transport compound,  
wherein the polyol is a polyester polyol represented by the formula:



where Ra and Rc independently represent linear alkyl groups or branched alkyl groups derived from polyols, Rb and Rd independently represent alkyl groups derived from polycarboxylic acids, and m, n, p, and q represent mole fractions of from 0 to 1, such that n+m+p+q=1,

wherein the charge transport compound is represented by:



2. The electrophotographic imaging member of claim 1, wherein the overcoating layer is formed from a solution comprising the film forming resin composition in a solvent.

3. The electrophotographic imaging member of claim 2, wherein the solution further comprises an acid catalyst.

4. The electrophotographic imaging member of claim 1, wherein the film forming resin composition comprises from about 5 to about 80 percent by weight of the charge transport compound, from about 5 to about 90 percent by weight of the polyol and from about 70 to about 5 percent by weight of the melamine compound.

5. The electrophotographic imaging member of claim 1, wherein the polyester polyol contains multiple pendent hydroxyl groups.

6. The electrophotographic imaging member of claim 1, wherein the melamine compound is a poly(melamine-formaldehyde) resin.

7. The electrophotographic imaging member of claim 1, wherein the melamine compound is an alkylated melamine-formaldehyde compound or resin, wherein the alkyl group possesses from about one to about four carbon atoms, or is a methoxymethylated melamine compound.

8. A process for forming an electrophotographic imaging member comprising:

providing an electrophotographic imaging member comprising a substrate, a charge generating layer, and a charge transport layer, and

25

forming thereover an overcoating layer comprising a cured film formed from a film forming resin composition comprising at least a melamine compound, a polyol, and a charge transport compound, wherein the polyol is a polyester polyol represented by the formula:



where Ra and Rc independently represent linear alkyl groups or branched alkyl groups derived from polyols, Rb and Rd independently represent alkyl groups derived from polycarboxylic acids, and m, n, p, and q represent mole fractions of from 0 to 1, such that  $n+m+p+q=1$ ,

wherein the charge transport compound is represented by:



9. The process of claim 8, wherein the forming step comprises: 30 providing a solution comprising the film forming resin composition in a solvent; coating the solution on the electrophotographic imaging member; and 35 crosslinking the film forming resin to form a cured polymeric film.

26

10. The process of claim 9, wherein the solution further comprises an acid catalyst.

11. The process of claim 8, wherein the polyester polyol contains multiple pendent hydroxyl groups.

12. An electrographic image development device, comprising an electrophotographic imaging member comprising:

a substrate,  
a charge generating layer,  
a charge transport layer, and  
an overcoating layer, said overcoating layer comprising a cured film formed from a film forming resin composition comprising at least a melamine compound, a polyol, and a charge transport compound, wherein the polyol is a polyester polyol represented by the formula:



where Ra and Rc independently represent linear alkyl groups or branched alkyl groups derived from polyols, Rb and Rd independently represent alkyl groups derived from polycarboxylic acids, and m, n, p, and q represent mole fractions of from 0 to 1, such that  $n+m+p+q=1$ ,

wherein the charge transport compound is represented by:



\* \* \* \* \*